

Patented Sept. 13, 1927.

1,642,349

## UNITED STATES PATENT OFFICE.

HARRY M. WILLIAMS AND ALFRED L. BOEGEHOOLD, OF DAYTON, OHIO, ASSIGNEES TO  
GENERAL MOTORS RESEARCH CORPORATION, OF DAYTON, OHIO, A CORPORATION  
OF DELAWARE.

## ALLOY STRUCTURE.

No Drawing.

Application filed April 13, 1923. Serial No. 633,012.

- The present invention relates to porous alloy structures and relates particularly to bearing materials composed entirely or largely of such porous alloys.
- 5 Among the objects of the present invention is to increase the strength of such alloys over that of similar materials heretofore produced while maintaining an equal or even greater porosity.
- 10 Another object of the invention is to render the process of producing the materials more economical and efficient and at the same time to produce a better material.
- With these and other objects, which will 15 appear hereinafter, the invention consists broadly in mixing a mass of fine metal particles with a smaller proportion of material that decomposes when heated, liberating a non-corrosive gas and leaving as a residue 20 a refractory material inert to the metallic particles and incapable of cohering to them, molding the mass under pressure to a desired form and then heating the molded form sufficiently to cause the metallic particles to 25 unite one to another and the other material to decompose, thereby producing a strong body of porous metal the pores or interstices of which contain particles of inert refractory filling material.
- 30 In applications, Serial Nos. 582,550 and 613,780 filed in the names of Harry M. Williams and Alfred L. Boegehold, processes of producing porous alloy articles have been described and claimed.
- 35 The present process is analogous to those processes already described but differs in that somewhat different materials are used and somewhat different processes. The analogy lies in the fact that powdered metals 40 and supporting filler are compressed together and the compressed article heated to an alloying temperature.
- In the present process as in the former ones, a mixture is made of finely divided metals, preferably copper and tin, in the proportions of 90 parts by weight of copper to 10 parts by weight of tin, and finely powdered non-alloying material. The so 45 prepared mixture is compressed into form in suitable dies under a pressure of around 50 75,000 to 80,000 pounds per square inch. After the compression step, the compressed article is packed in carbonaceous material and heated to a temperature of about 1350° F. for a period of about five hours. After 55 the article has become cool enough to handle, it is removed from the carbonaceous packing and, if a bushing, is sized, for example, by forcing through a die upon a mandrel. This latter operation simultaneously sizes the bushing, both inside and outside.
- In the present process, instead of the non-alloying materials mentioned in these former applications, namely, graphite, mica, soap 60 stone, talc, etc., a material is used which, under the conditions of the process, is decomposed with liberation of a non-corrosive volatile substance leaving as a residue a material inert to the other constituents present 65 and capable of acting as a supporting filler for the bearing material. For this purpose, a number of classes of materials may be used and among these classes are the carbonates (including the bicarbonates and basic carbonates), hydrates or hydroxides (e. g., calcium hydroxide), nitrates (e. g., copper nitrate), etc., of the metals. All materials of 70 these classes which fulfill the conditions just mentioned, upon decomposing, leave behind metal oxides to act as the supporting filler. However, the material preferred to be used is magnesium carbonate. This material in the heating step becomes decomposed giving 75 off carbon dioxide leaving magnesium oxide behind.
- The magnesium oxide acts as an excellent supporting filling material for the bearing and the carbon dioxide being liberated in the interstices between the metal particles tends to increase the porosity of the finished article and also apparently assists in the alloying, probably because of the non-oxidizing character of the gas under those conditions.
- 80 A specific example of the proportions used in making the preferred form of bearing 85

coming within the present invention is the following:

|                     | Parts by weight: |
|---------------------|------------------|
| Copper powder       | 90               |
| Tin powder          | 10               |
| Magnesium carbonate | 4                |

These materials in very finely divided condition are intimately mixed and compressed under a pressure of 75,000 to 80,000 pounds per square inch, the article thus formed, heated for five or six hours to a temperature of 1350° F. and properly finished, produces a, for example, bearing bushing which is capable of absorbing well over one percent by weight of oil and one which is quite high in strength and has a very long life even under quite trying conditions.

Another example, one in which the porosity is increased by making use of a process of one of the prior applications, is as follows:

|                     | Parts by weight: |
|---------------------|------------------|
| Copper powder       | 90               |
| Tin powder          | 10               |
| Salicylic acid      | 2                |
| Magnesium carbonate | 3½               |

In this latter example, the salicylic acid volatilizes in the heating step and thus, in addition to the porosity caused by the elimination of carbon dioxide, very greatly increases the porosity of the final product.

The bearings having these proportions of constituents are capable of absorbing close to five percent by weight of oil.

Magnesium carbonate has been mentioned as the preferred non-alloying material for use in carrying out the present invention, and the description confined largely to this substance, but it should be understood that the invention is not limited to it, as many other substances, as indicated above, have been used to make satisfactory bearing materials. Magnesium carbonate has been chosen as the most preferable one because of the fact that it liberates gaseous carbon dioxide upon being heated leaving a residue which serves as an excellent supporting filler. Another advantage in the use of magnesium carbonate is that it works well in the compression dies.

Further, while the description has been confined chiefly to the preferred processes and compositions it should be understood that other processes and compositions might be adopted all of which come within the scope of the claims which follow.

What we claim is as follows:

1. The process of producing bearing materials which comprises intimately mixing finely divided alloyable metals and a finely divided non-alloying material of itself

capable of decomposing at high temperature to give off a non-corrosive volatile substance and to leave, as the result of its disintegration, a residue capable of acting as a supporting filler for the bearing material; compressing the mixture; and heating under non-oxidizing conditions to cause the said decomposition and also alloying of the metals.

2. The process of producing bearing materials which comprises intimately mixing finely divided copper and tin and a finely divided non-alloying material of itself capable of decomposing at high temperature to give off a non-corrosive volatile substance and to leave, as the result of its disintegration, a residue capable of acting as a supporting filler for the bearing material; compressing the mixture; and heating under non-oxidizing conditions to cause the said decomposition and also alloying of the metals.

3. The process of producing bearing materials which comprises intimately mixing finely divided alloyable metals and finely divided magnesium carbonate; compressing the mixture; and heating under non-oxidizing conditions to cause decomposition of the carbonate and also alloying of the metals.

4. The process of producing bearing materials which comprises intimately mixing finely divided copper and tin and a finely divided magnesium carbonate; compressing the mixture; and heating under non-oxidizing conditions to cause decomposition of the carbonate and also alloying of the metals.

5. The process of producing porous metallic structures capable of retaining liquid in the pores, which consists of intimately mixing fine particles of metal capable of uniting when subjected to relatively high temperatures, with a finely divided material incapable of cohering to said particles of metal, but capable of decomposing at said relatively high temperatures to give off a non-corrosive volatile substance and leaving a residue which functions as a supporting filler for the metallic mass when union of the particles has been effected; compressing said mixture into a mass of the desired form and heating the form sufficiently to effect union of the metallic particles and decomposition of the material mixed with them.

6. The process of producing porous metal structures capable of retaining liquid in the pores, which consists of intimately mixing fine particles of metal capable of uniting when subjected to relatively high temperatures, with finely divided magnesium carbonate, compressing said mixture into a mass of the desired form and heating the form sufficiently to effect union of the metallic particles and decomposition of the magnesium carbonate.

7. A bearing material comprising an alloy having uniformly distributed therethrough

a metal oxide and having a capacity for absorption of oil in amounts exceeding one percent of its weight.

8. A bearing material comprising an alloy having uniformly distributed therethrough magnesium oxide and having a capacity for absorption of oil in amounts exceeding one percent of its weight.

9. A bearing material comprising a bronze

having uniformly distributed therethrough 10 magnesium oxide and having a capacity for absorption of oil in amounts exceeding one percent of its weight.

In testimony whereof we hereby affix our signatures.

HARRY M. WILLIAMS.

ALFRED L. BOEGEHOOLD.